

## 1

2,752,311

**LUBRICANT CONTAINING A METAL DERIVATIVE  
OF A HYDROXYARYLALKYL POLYAMINE AND  
A METAL DITHIOCARBAMATE**

Frederic C. McCoy and James M. Caffrey, Jr., Beacon, N. Y., and William R. Hencke, Old Tappan, N. J., assignors to The Texas Company, New York, N. Y., a corporation of Delaware

No Drawing. Application July 26, 1952,  
Serial No. 301,162

3 Claims. (Cl. 252—33.6)

The present invention relates to improved lubricating compositions obtained by means of a new combination of additives. More particularly, the invention relates to mineral lubricating oils containing metal derivatives of hydroxyarylalkyl polyamines in conjunction with metal dithiocarbamates.

When hydrocarbon oils are employed as lubricants in internal combustion engines, they tend to undergo oxidation and other deterioration under the severe conditions to which they are subjected, including high temperatures for long periods of time and the presence of catalytic metal surfaces. As a result of this deterioration, acids are produced which are corrosive to the bearings and other engine parts, and gums and sludges are formed which cause ring sticking and otherwise reduce the efficiency of operation of the engine. It is, therefore, common practice to add to lubricating oils small amounts of compounds which have the property of imparting improved oxidation stability and/or anti-corrosiveness, and also compounds of the "detergent" type, which act to reduce the formation of gums and sludges or to disperse and alter the character thereof so as to reduce the formation of varnish-like deposits upon the lubricated engine parts.

However, many additives which are employed to improve certain properties of a lubricating oil have been found to exert a deleterious effect upon other properties of the oil, and also the effectiveness of an additive is frequently diminished or destroyed when it is employed in a lubricating oil together with other additives of different chemical type. Since a catalytic effect is involved between the additives themselves as well as between the additives and the oil, the effect obtainable by the use of two or more additives in combination cannot be predicted on the basis of their separate effects in lubricating compositions.

It has now been found, in accordance with the present invention, that lubricating compositions of very special properties, including excellent oxidation resistance and anti-corrosiveness to metals in addition to very superior detergency characteristics, are obtained by adding to hydrocarbon lubricating oils a minor proportion of a metal derivative of a hydroxyarylalkyl polyamine, and a minor proportion of a metal salt of a hydrocarbon-substituted dithiocarbamate.

By the cooperative effect of the above additives a superior detergency is produced, and in addition the oxidation tendency and corrosiveness of the composition are effectively inhibited. The oxidation inhibiting action of the dithiocarbamate involves an inhibiting effect upon the hydroxyarylalkyl polyamine derivative, since compounds

## 2

of the latter type are normally strong pro-oxidants in lubricating compositions. The effectiveness of the dithiocarbamates as both oxidation and corrosion inhibitors in these lubricating compositions containing hydroxyarylalkyl polyamine derivatives is very unexpected in view of the ineffectiveness for this purpose of a large number of other compounds commonly employed as oxidation and corrosion inhibitors in lubricating compositions, including various other sulfur-containing compounds.

10 The metal derivatives of hydroxyarylalkyl polyamines contemplated by this invention are the metal derivatives of condensation products disclosed in U. S. 2,353,491, and also the corresponding hydroxy-metal and alkoxy-metal derivatives of such condensation products, where-  
15 in the alkoxy group contains from 1 to 5 carbon atoms, as disclosed and claimed in the copending application of H. D. Kluge and F. W. Moore, Serial No. 287,266, filed May 10, 1952, now Patent No. 2,725,357. These com-  
pounds are obtained by interreacting a hydroxyaromatic compound with an aliphatic aldehyde and with an aliphatic  
20 polyamine containing at least two reactive, i. e., primary or secondary, amine groups, so as to form a condensation product, and then further reacting the condensation product thus obtained so as to replace the hydroxyl hydrogen  
25 with a member of the group consisting of metal, hydroxy-  
metal groups and lower alkoxy-metal groups. The hydroxyaromatic compound preferably contains an aliphatic hydrocarbon group of sufficient size to impart oil-solubility to the final product. While either mono- or poly-  
30 nuclear hydroxyaromatic compounds may be employed in forming the condensation products, as discussed in the above-cited patent, the hydroxyaromatic compound em-  
ployed is most suitably phenol, containing at least one aliphatic hydrocarbon group containing from about 5 to  
35 30 carbon atoms.

The product obtained by the above condensation re-  
action has been found by analysis to consist principally of compounds wherein one hydrogen attached to each nitro-  
gen atom of the primary or secondary amine groups is  
40 replaced by a hydroxyarylalkyl group, with smaller amounts of both higher and lower condensation products. For example, when ethylene diamine is employed as the amine reactant, the product consists predominantly of N,N'-bis(hydroxyarylalkyl)-1,2-diamines. In forming the additive for use according to this invention, the condensa-  
45 tion product is preferably converted directly to the metal derivative, although a prior separation may be carried out if desired to remove any higher or lower condensation products.

Because of the generally superior detergency character-  
50 istics of compounds of the alkaline earth metals and zinc, the metal employed in forming the above metal derivatives is preferably chosen from this group, although other metals such as the alkali metals, tin, lead, etc., may be employed if desired. With particular advantage, when the compounds are to be employed as additives where the character of the combustion chamber deposits is an im-  
portant consideration, the metal is chosen from the group consisting of magnesium and zinc. For regular heavy  
55 motor oils, however, the heavier metals such as calcium and barium may be suitably employed.

The metal dithiocarbamates which are employed as the second component of the additive combination of our invention are polyvalent metal salts of organic-substituted dithiocarbamic acids, such as described for example in

U. S. 2,400,106. They are preferably polyvalent metal salts of aliphatic hydrocarbon-substituted dithiocarbamic acids, wherein the aliphatic hydrocarbon groups contain a total of at least 8 carbon atoms. Compounds of this class wherein the metal is a member of the group consisting of the alkaline earth metals and zinc, and particularly of the group consisting of magnesium and zinc, are especially desirable. As examples of suitable compounds of this class may be mentioned zinc dibutyl dithiocarbamate, 10 tin diamyl dithiocarbamate, zinc di(2-ethylhexyl) dithiocarbamate, calcium octyl-butyl dithiocarbamate, magnesium methyl-octyl dithiocarbamate, aluminum dioctyl dithiocarbamate, zinc "petroleum base" dithiocarbamates, nickel dicetyl dithiocarbamate, and so forth.

In addition to the compounds discussed above, the lubricating compositions of this invention preferably contain also an additive selected from the class of compounds consisting of polyvalent metal salts of alkylated hydroxy-aromatic monocarboxylic acids, as disclosed for example in U. S. 2,477,913. The hydroxyaromatic monocarboxylic acids may be either mono- or poly-nuclear, such as for example aliphatic hydrocarbon substituted-salicylic, ortho hydroxy naphthoic and anthracene ortho hydroxy carboxylic acids. Of the polyvalent metals which may be employed to form the salts of these acids, preference is given to metals of the group consisting of the alkaline earth metals and zinc, and particularly to magnesium and zinc. As particularly suitable compounds of this class may be mentioned the calcium, barium, magnesium, and zinc salts of alkyl (C<sub>5</sub>-30) salicylic acid. If desired, these salts may be partially in the form of their "inner ring" salts, as described in U. S. 2,293,419.

The compounds of the above described classes of lubricant additives may be employed in hydrocarbon lubricating oils in varying amounts, ranging from very small amounts up to amounts representing the limits of their solubilities. For ordinary purposes, the amount of each additive employed will lie within the range of from about 0.1 to about 5.0 per cent, and preferably within the range of from about 0.25 to about 2.0 per cent by weight of the lubricating composition.

The hydrocarbon oils compounded according to this invention will usually be petroleum fractions of lubricating viscosity, including highly refined and moderately refined oils from paraffinic, naphthenic and mixed base crude oils. However, synthetic oils, such as various polymer oils of lubricating viscosity, may also be employed if desired.

The superior lubricating properties obtained by use of the additive combinations of our invention have been demonstrated in numerous tests, including both laboratory bench tests and engine tests. Results obtained upon lubricating oils containing typical compounds of each of the hereinabove described classes of compounds in the combinations contemplated by our invention are described in the following examples.

As representative of the class of additives consisting of metal derivatives of hydroxyaryalkyl polyamines, the magnesium, methoxy-magnesium and barium derivatives of condensation products obtained by interreacting alkyl phenols with formaldehyde and with ethylene diamine were employed in these tests. The alkyl phenols employed comprised chiefly para-alkyl substituted phenols, which upon condensation with ethylene diamine formed N,N'-bis(2-hydroxy-5-alkyl-benzyl)-1,2-diamino ethanes. The magnesium and methoxy-magnesium derivatives of these compounds were obtained as described in the aforementioned application of Kluge and Moore, Serial No. 287,266, by first interreacting an alkyl phenol with formaldehyde and with ethylene diamine, and then treating the condensation product thus obtained with magnesium methylate, employing equimolar proportions of condensation product and magnesium methylate to obtain the normal magnesium salt and at least 2 mols of magnesium methylate per mole of condensation product to obtain

the methoxy-magnesium derivative. As described in the examples given in the above application, the condensation reaction was carried out by adding the reactants together in an ethanol solution while the temperature was maintained below about 95° F. and then refluxing for several hours to complete the reaction, employing approximately equimolar proportions of alkyl phenol and formaldehyde and about one half mol proportion of ethylene diamine. The barium derivative was prepared from a condensation product obtained as described above by reacting the condensation product with barium hydroxide in benzene solution, employing equimolar proportions of condensation product and barium hydroxide.

The dithiocarbamate salt employed in the tests was a commercial zinc dibutyl dithiocarbamate, which is sold by the R. T. Vanderbilt Co. under the trade name of "Butyl Zimate." This product had a melting point of 106° F., a sulfur content of 28.25 per cent and a zinc content of 14.3 per cent.

20 The zinc alkyl salicylate which was employed in the tests was obtained by carboxylating an alkyl phenol and then converting the alkyl salicylic acid thus obtained to the zinc salt by reacting it with zinc acetate,



The alkyl phenol employed in the carboxylation was a product having a hydroxyl number of 135 and a molecular weight of 413, indicating that it contained an average of 23 alkyl carbon atoms per molecule. The carboxylation was carried out by reacting the sodium salt of this alkyl phenol with carbon dioxide under 300 p. s. i. g. pressure and at a temperature of 325° F. until the phenol was substantially entirely reacted. The reaction of the alkyl salicylic acid with zinc acetate was carried out by heating the reactants together in xylene solution under reflux, employing one mole of zinc acetate per two moles of alkyl salicylic acid, and thereafter distilling off the water and/or acetic acid of reaction and the solvent. The product, which was finally obtained in the form of a 25 per cent solution of the zinc alkyl salicylate in a lubricating oil of 300 S. S. U. viscosity at 100° F., analyzed 1.74 per cent zinc, as compared with the theoretical value of 1.66 per cent.

#### EXAMPLE 1.—CORROSION TEST

Table I below gives the results obtained in the Mac-Coull Corrosion Test upon a mineral lubricating oil containing the additive combinations of our invention, comparatively with those obtained upon the same oil containing the additives of these combinations separately and also in combination with various other additives. This test is an empirical test designed to show the corrosiveness and oxidation stability of a lubricating oil under the bearing lubrication conditions existing in an internal combustion engine. The procedure is fully described in SAE Transactions, v. 50, pp. 338-345 (August 1942). Briefly, it comprises rotating a copper-lead bearing specimen at high speed in a sample of the test oil maintained at 350° F. in the presence of catalytic metal surfaces and of air, and determining the loss in weight of the bearing specimen at two hour intervals up to ten hours. The mineral lubricating oil employed was a low-sulfur oil having an SUS viscosity at 100° F. of about 518, obtained by solvent refining and clay and acid treating a wax distillate fraction from a paraffin base crude oil. It contained 1.76 percent of a mixture of high molecular weight methacrylate polymers employed in lubricating oils as viscosity improving agents.

70 For convenience, derivatives of phenol-formaldehyde-ethylene diamine condensation products are referred to in the tables as derivatives of N,N'-bis(hydroxy-alkyl-benzyl)-1,2-diamino ethanes, which were found by analysis to comprise the chief component of these condensation products.

Wherever possible, the values for duplicate runs on each lubricating composition have been given in the tables, as an indication of the reproducibility and reliability of the results.

TABLE I  
*MacCoull corrosion test at 350° F.*

| Detergent                                                                                                                     | Inhibitor                                                | Weight Loss, mg./10 hrs. | Neutralization No. Used oil |
|-------------------------------------------------------------------------------------------------------------------------------|----------------------------------------------------------|--------------------------|-----------------------------|
| None                                                                                                                          | None                                                     | 141; 180                 | 13.2; 12.5                  |
| 1% Mg derivative of N,N'-bis(hydroxy-alkyl) (C <sub>22</sub> ) benzyl)-1,2-diamino ethane.                                    | do                                                       | 63; 42                   | 13.3; 13.2                  |
| 1% Zn alkyl salicylate                                                                                                        | do                                                       | 69; 61                   | 5.3; 5.2                    |
| None                                                                                                                          | 1% Butyl Zimate                                          | 6; 4 (115) <sup>1</sup>  | 1.1 (6.7) <sup>1</sup>      |
| 1% Mg derivative of N,N'-bis(hydroxy-alkyl) (C <sub>22</sub> ) benzyl)-1,2-diamino ethane + 0.5% Zn alkyl salicylate.         | None                                                     | 142; 125                 | 13.3; 12.7                  |
| Do                                                                                                                            | 0.5% Butyl Zimate                                        | 1; 1                     | 0.08                        |
| Do                                                                                                                            | 1% Santolube 394-C <sub>2</sub>                          | 108; 145                 | 7.7; 7.8                    |
| 1% Methoxy-Mg derivative of N,N'-bis(hydroxy-alkyl) (C <sub>16</sub> ) benzyl)-1,2-diamino ethane.                            | None                                                     | 25; 22                   | 5.4; 5.5                    |
| 1% Methoxy-Mg derivative of N,N'-bis(hydroxy-alkyl) (C <sub>22</sub> ) benzyl)-1,2-diamino ethane.                            | 0.5% Butyl Zimate                                        | 2; 9                     | 0.44                        |
| 1% Methoxy-Mg derivative of N,N'-bis(hydroxy-alkyl) (C <sub>22</sub> ) benzyl)-1,2-diaminoethane + 1% Zn alkyl salicylate.    | None                                                     | 105; 112                 | 10.2; 10.9                  |
| 1% Methoxy-Mg derivative of N,N'-bis(hydroxy-alkyl) (C <sub>22</sub> ) benzyl)-1,2-diaminoethane + 0.5% Zn alkyl salicylate.  | do                                                       | 79; 100                  | 10.5                        |
| Do                                                                                                                            | Lubrizol 747 <sup>2</sup>                                | 86; 25                   | 7.7; 7.9                    |
| 1% Methoxy-Mg derivative of N,N'-bis(hydroxy-alkyl) (C <sub>22</sub> ) benzyl)-1,2-diamino ethane + 1% Zn alkyl salicylate.   | 0.5% Butyl Zimate                                        | 3; 2                     | 0.77 alk.                   |
| 1% Methoxy-Mg derivative of N,N'-bis(hydroxy-alkyl) (C <sub>22</sub> ) benzyl)-1,2-diamino ethane + 0.5% Zn alkyl salicylate. | do                                                       | 1; 1                     | 0.44                        |
| Do                                                                                                                            | 1% di-2-ethylhexyl ether of dithiodiglycol.              | 147; 131                 | 10.4                        |
| Do                                                                                                                            | 1% di-2-ethylhexyl disulfide.                            | 100; 107                 | 8.2; 8.7                    |
| Do                                                                                                                            | 1% isophorone-mercaptan condensation product.            | 141; 132                 | 6.2; 5.9                    |
| Do                                                                                                                            | 1% 2-ethyl-hexyl thiocellosolve.                         | 96; 98                   | 8.8; 9.2                    |
| Do                                                                                                                            | 1% dibenzyl disulfide.                                   | 102; 71                  | 7.9; 7.7                    |
| Do                                                                                                                            | 1% 4-methyl-2-tert. butyl-6-tert. amyl thiomethylphenol. | 142; 131                 | 10.5; 11.0                  |

<sup>1</sup> A different base oil giving a weight loss of 115 mg. and a neutralization No. of 6.7 was used in this test.

<sup>2</sup> A commercial oxidation and corrosion inhibitor consisting of oxidation product of olefin-phosphorus pentasulfide reaction product, obtained from the Monsanto Chemical Co.

<sup>3</sup> A commercial oxidation and corrosion inhibitor comprising the barium salt of an alcohol-P<sub>2</sub>S<sub>5</sub> reaction product, obtained from the Lubrizol Corp.

As shown by the above table, only a moderate improvement in the corrosion inhibiting properties of a mineral lubricating oil was obtained by use of a metal derivative of a hydroxy-arylkyl polyamine or of a metal salt of a hydroxyaromatic acid, employed separately. A very corrosive oil, substantially equivalent to the uncompounded oil, was produced when compounds of both of these classes of compounds were employed in combination. Furthermore, the corrosiveness of lubricating oils containing these additives in combination was not inhibited by the use of a number of other compounds commonly employed in lubricating compositions as oxidation and corrosion inhibitors, including various sulfur-containing compounds. However, by the addition of a small amount of a metal dithiocarbamate to lubricating oils containing a metal derivative of a hydroxyarylkyl

polyamine, either alone or in combination with a metal hydroxyaromatic acid salt, lubricating oils of very exceptional anti-corrosiveness and oxidation stability were obtained.

### EXAMPLE 2.—DETERGENCY TESTS

Table II below shows the detergency characteristics imparted to a lubricating oil by use of the additive combinations of this invention, comparatively with the detergent effectiveness of the same additives employed separately. The Toettcher varnish test and the High Temperature Deposits Test of the table are bench tests which have been found to correlate well with the lacquer forming and the oil ring sticking characteristics of a motor oil in actual service. In the Toettcher varnish test, a weighed glass cylinder is immersed in a sample of the test oil maintained at 350° F. and agitated by a centrifugal mixer. Copper baffles are also immersed in the test oil to act as oxidation catalysts. After 13 hours the test is terminated and the glass cylinder removed, washed with pentane, dried and reweighed. The amount of varnish deposited on the cylinder is the difference between the initial and final weights of the cylinder. The neutralization number of the used oil is also determined. The High Temperature Deposits Test is carried out by repeatedly dipping an aluminum cylinder one inch in diameter and three inches long, maintained at 525° F. into a beaker containing a sample of the test oil, for a period of 20 hours. The test specimen is then washed with pentane and dried, and the weight of deposits found by the increase in weight. The test specimen is then brushed to remove loose deposits and reweighed to determine the amount of varnish-like deposits. A lubricating oil of the same type as that employed in the corrosion test of Example 1 was employed in these tests.

TABLE II

### Detergency tests

| Additive                                                                                                                                        | Toettcher Varnish Test, 350° F. |                            | High Temperature Deposits Test, 525° F. |          |
|-------------------------------------------------------------------------------------------------------------------------------------------------|---------------------------------|----------------------------|-----------------------------------------|----------|
|                                                                                                                                                 | Weight of deposits, mg.         | Neutralization N. Used oil | Total                                   | Adherent |
| None (base oil)                                                                                                                                 | 15.2                            | 6.0                        | 452                                     | 326      |
| 1% Mg derivative of N,N'-bis(hydroxy-alkyl) (C <sub>22</sub> ) benzyl)-1,2-diamino ethane + 0.5% Zn alkyl salicylate                            | 3.2; 4.1                        | 9.5; 9.8                   | 159; 78                                 | 19; 11   |
| 0.5% Butyl Zimate                                                                                                                               | 4.1; 4.4                        | 9.0; 9.3                   | 1; 1                                    | 1; 1     |
| 1% Mg derivative of N,N'-bis(hydroxy-alkyl) (C <sub>16</sub> ) benzyl)-1,2-diamino ethane + 0.5% Zn alkyl salicylate + 0.5% Butyl Zimate        | 0.0; 0.1                        | 0.05 alk.                  | 162; 117                                | 4        |
| 1% Methoxy-Mg derivative of N,N'-bis(hydroxy-alkyl) (C <sub>22</sub> ) benzyl)-1,2-diaminoethane + 0.5% Zn alkyl salicylate + 0.5% Butyl Zimate | 0.2; 0.7                        | 0.12 alk.                  | 1                                       | 1        |

As shown by the data given in the above table, lubricating compositions obtained by use of additive combinations of this invention had outstandingly superior detergency characteristics. The detergency effect of the additives employed in combination was superior to that obtained by any of the additives employed separately, and in addition the oxidation tendency of the composition, including the oxidation-promoting effects of both the magnesium derivatives of N,N'-bis(2-hydroxy-5-

alkyl(C<sub>22</sub>)benzyl)1,2-diamino ethane and the zinc salicylate, were very effectively inhibited.

#### EXAMPLE 3.—THE ENGINE TESTS

In addition to the above laboratory tests, engine tests were carried out upon the compounded oils of this invention to determine their performance under actual operating conditions. These compounded oils were obtained by adding typical compounds of our additive combinations to a lubricating oil of the same type as that employed in the tests described in Examples 1 and 2.

Table II below gives the results obtained in the Lauson L-4 Engine Test. This test was carried out by employing the test oils to lubricate a single cylinder standard Lauson engine while it was operated for 40 hours at 1850 revolutions per minute, with the jacket temperature maintained at 200° F. and the sump temperature at 310° F. At the end of the run the engine was taken down and inspected for bearing weight loss and piston deposits. A bearing weight loss of less than 200 mg. in this test is considered satisfactory and a loss of less than 100 mg. is considered excellent. The pistons were rated on a scale of from 0 for a completely varnished piston to 10 for a completely clean piston. A piston rating above 8 indicates an oil of satisfactory detergency, while a rating of 9 or more indicates an oil of very excellent detergency.

TABLE III  
Lauson L-4 engine test

| Additive                                                                                                                                   | Bearing Weight Loss, mg. | Piston Rating | Neutralization No. Used oil |
|--------------------------------------------------------------------------------------------------------------------------------------------|--------------------------|---------------|-----------------------------|
| None (base oil)                                                                                                                            | 694                      | 8.0           | 6.7                         |
| 1% Methoxy-Mg derivative of N,N'-bis(hydroxy-alkyl(C <sub>22</sub> )benzyl)-1,2-diamino ethane+1% Zn alkyl salicylate                      | 359                      | 8.1           | 6.0                         |
| 1% Methoxy-Mg derivative of N,N'-bis(hydroxy-alkyl(C <sub>22</sub> )benzyl)-1,2-diamino ethane+0.5% Butyl Zimate                           | 185                      | 8.3           | 4.3                         |
| 1% Methoxy-Mg derivative of N,N'-bis(hydroxy-alkyl(C <sub>22</sub> )benzyl)-1,2-diamino ethane+0.5% Zn alkyl salicylate+0.75% Butyl Zimate | 34                       | 9.6           | 3.1                         |
| 1% Methoxy-Mg derivative of N,N'-bis(hydroxy-alkyl(C <sub>22</sub> )benzyl)-1,2-diamino ethane+0.5% Zn alkyl salicylate+0.5% Butyl Zimate  | 148                      | 9.0           | 3.0                         |
| 1% Mg derivative of N,N'-bis(hydroxy-alkyl(C <sub>22</sub> )benzyl)-1,2-diamino ethane+0.5% Zn alkyl salicylate+0.5% Butyl Zimate          | 93                       | 9.7           | 2.1                         |
| 1.1% Ba derivative of N,N'-bis(hydroxy-alkyl(C <sub>22</sub> )benzyl)-1,2-diamino ethane+0.5% Zn alkyl salicylate+0.5% Butyl Zimate        | 137                      | 9.3           | 3.4                         |

As shown by the data given in the above table, a lubricating composition having both satisfactory detergency and anti-corrosiveness was obtained by the use of a small amount of a hydroxyarylalkyl polyamine metal derivative and a small amount of a dithiocarbamate salt in a lubricating oil. The data also show that, very unexpectedly, a pronounced synergistic effect upon both the detergency and the anti-corrosiveness of the lubricating composition under the conditions of this test were obtained when a small amount of a metal salicylate was also added to the composition containing the above additive combination.

Table IV below also shows the superior detergency properties of the compounded lubricants of this invention when employed in the lubrication of a heavy duty diesel engine, in comparison with those of a commercial diesel oil of good grade. This test was carried out by operating a super-charged single cylinder 5 $\frac{1}{4}$  by 8 inch Caterpillar diesel test engine for 50 hours, with an engine speed of 900 revolutions per minute, a fuel-oil ratio of 0.055 and a crankcase oil temperature of 200° F. At the end of each run the power section of the engine was inspected for deposits and other conditions detrimental to engine operation, and rated by a demerit rating system. Accord-

ing to this system, a rating of 183 is accorded to the worst possible condition for total piston deposit demerits in this test, while zero represents a new or clean condition. For ring sticking, the worst possible condition would be assigned a rating of 240.

TABLE IV  
Caterpillar diesel engine test

| Additive                                                                                                                                   | Demerit Rating of Piston Assembly |                        | Neutralization No. Used oil |
|--------------------------------------------------------------------------------------------------------------------------------------------|-----------------------------------|------------------------|-----------------------------|
|                                                                                                                                            | Total piston Deposit Demerits     | Ring Sticking Demerits |                             |
| Commercial Diesel Oil                                                                                                                      | 45                                | 0                      | 1.02                        |
| 1% Methoxy-Mg derivative of N,N'-bis(hydroxy-alkyl(C <sub>22</sub> )benzyl)-1,2-diamino ethane+0.5% Zn alkyl salicylate+0.75% Butyl Zimate | 23                                | 0                      | 0.10                        |
| 1% Mg Derivative of N,N'-bis(hydroxy-alkyl(C <sub>22</sub> )benzyl)-1,2-diamino ethane+0.5% Zn alkyl salicylate+0.5% Butyl Zimate          | 19                                | 0                      | 0.09                        |
| 1.1% Ba derivative of N,N'-bis(hydroxy-alkyl(C <sub>22</sub> )benzyl)-1,2-diamino ethane+0.5% Zn alkyl salicylate+0.5% Butyl Zimate        | 38                                | 30                     | 0.62                        |

Table V gives results obtained upon a typical compounded oil of our invention in a 40-hour Chevrolet engine test designed to measure the varnish-forming properties of an oil under severe conditions. This test was carried out with a standard Chevrolet engine operated at a speed of 2,500 revolutions per minute and a crankcase oil temperature of 275° F., employing as the fuel an unleaded 420° F. end point thermally cracked naphtha. The oil employed in this test was a lubricating oil of the same type as described in connection with the previous tests compounded with 1% of the methoxy-magnesium derivative of N,N'-bis(2-hydroxy-5-alkyl(C<sub>22</sub>)-benzyl)-1,2-diamino ethane, 0.5% of Zn alkyl salicylate and 0.5% of Butyl Zimate.

TABLE V  
Chevrolet engine test

|                                | Compounded Oil | Base Oil |
|--------------------------------|----------------|----------|
| Piston Skirt Deposits, mg.     | 62             | 507      |
| Oil Ring deposits, mg.         | 126            | 772      |
| Pan and cover deposits, mg.:   |                |          |
| Acetone soluble                | 87             | 2,176    |
| Acetone insoluble              | 794            | 2,546    |
| CRC ratings:                   |                |          |
| Piston                         | 10.0           | 5.5      |
| Total                          | 92             | 70       |
| Used oil tests:                |                |          |
| Neutralization number—         |                |          |
| 0 hours                        | 0.05           | 0.05     |
| 40 hours                       | 0.69           | 5.0      |
| Viscosity, SUS, at 210° F.—    |                |          |
| 0 hours                        | 55.4           | 53.3     |
| 40 hours                       | 56.6           | 72.3     |
| Dissolved sludge, mg./10 g.—   |                |          |
| 0 hours                        | None           | None     |
| 40 hours                       | 20             | 422      |
| Undissolved sludge, mg./10 g.— |                |          |
| 0 hours                        | 13             | None     |
| 40 hours                       | 33             | 223      |

The data given in the above table show the very excellent detergency characteristics of a typical compounded lubricant of this invention obtained in actual operation of an internal combustion engine.

Obviously many modifications and variations of the invention, as hereinbefore set forth, may be made without departing from the spirit and scope thereof and, therefore, only such limitations should be imposed as are indicated in the appended claims.

We claim:

1. A lubricant composition comprising a major proportion of a mineral lubricating oil having admixed therewith about 0.1-5.0 per cent by weight based on the weight of

the composition of the methoxy magnesium derivative of N,N'bis(2-hydroxy-5-alkyl(C<sub>15-30</sub>)benzyl) - 1,2 - diamino ethane and about 0.1-5.0 per cent by weight based on the weight of the composition of zinc dibutyl dithiocarbamate.

2. A lubricant composition comprising a major proportion of a mineral lubricating oil having admixed therewith about 0.1-5.0 per cent by weight based on the weight of the composition of a compound chosen from the class consisting of magnesium and methoxy magnesium derivatives of N,N'bis(2-hydroxy-5-alkyl(C<sub>15-30</sub>)-benzyl)-1,2-diamino ethane, about 0.1-5.0 per cent by weight based on the weight of the composition of zinc dibutyl dithiocarbamate and about 0.1-5.0 per cent by weight based on the weight of the composition of zinc alkyl (C<sub>15-20</sub>) salicylate.

3. A lubricant composition comprising a major proportion of a mineral lubricating oil having admixed therewith about 0.1-5.0 per cent by weight based on the weight of the composition of the methoxy magnesium derivative of N,N'bis(2-hydroxy-5-alkyl(C<sub>15-30</sub>)benzyl) - 1,2 - diamino ethane, about 0.1-5.0 per cent by weight based on the weight of the composition of zinc dibutyl dithiocarbamate and about 0.1-5.0 per cent by weight based on the weight of the composition of zinc alkyl (C<sub>15-20</sub>) salicylate.

## References Cited in the file of this patent

## UNITED STATES PATENTS

|           |                |       |               |
|-----------|----------------|-------|---------------|
| 2,353,491 | Oberright      | ----- | July 11, 1944 |
| 2,477,913 | Van Loon       | ----- | Aug. 2, 1949  |
| 2,400,106 | Denison et al. | ----- | May 14, 1946  |